# EUROPEAN PATENT SPECIFICATION

(11) **EP 1 760 727 B1**
(45) Date of publication and mention of the grant of the patent: **07.01.2015**
(21) Application number: 05291837.2
(22) Date of filing: 06.09.2005
(51) Int. Cl.: H01B 13/00, H01B 11/18, H01P 11/00

(54) **Process and apparatus for manufacturing structures guiding electromagnetic waves**
Verfahren und Vorrichtung zum Herstellen von elektromagnetischen Wellenleiterstrukturen
Procédé et dispositif pour la formation de structures permettant de guider des ondes électromagnétiques

(43) Date of publication of application: 07.03.2007
(73) Proprietor: ALCATEL LUCENT, 92100 Boulogne-Billancourt (FR)
(72) Inventor: Greiner, Martin, 30966 Hemmingen (DE); Mahlandt, Erhard, 30880 Laatzen (DE); Mientkewitz, Olaf, 30952 Ronnenberg (DE)
(74) Representative: Wetzel, Emmanuelle

(56) References cited:
- EP-A- 0 484 533
- GB-A- 304 192
- US-A- 4 773 976
- US-A1- 2004 026 111
- US-A1- 2004 055 153

## Description

The present invention relates generally to structures guiding electromagnetic waves and particularly to telecommunication cables comprising a conductive layer for transmission of radio frequency waves and a manufacturing method thereof.

Coaxial cables and other radio frequency cables are known in the art for transmitting high frequency signals. A conventional coaxial cable is formed out of an inner conductor, a dielectric material, and an outer conductor. The conductors may be tubular or solid. The two conductors are made of metal or another electrically conductive material and are disposed concentrically with the dielectric material disposed between the two. If necessary, one or more additional protective coatings of an electrically insulating material can be provided on the outer conductor.

As it is known in the art, at radio frequencies, particularly at frequencies above 1 MHz, the current flowing through the cable conductors tends to flow only directly beneath the surfaces of said conductors. This is commonly known as a "skin effect". More particularly, current flows through and directly beneath an inside surface of the outer conductor and an outside surface of the inner conductor.

Each conductor may be manufactured by known methods. For example US Patent 6,717,493 discloses a radio frequency coaxial cable with clad conductors formed in the same manner. The tubular conductors are formed from a sheet of two strips of material, a base layer formed of a relatively higher conductivity material and a bulk layer formed of a relatively lower conductivity material. The higher conductivity material may be copper while the lower conductivity material may be aluminium. To form either the inner conductor and the outer conductor the sheet is folded or curved and the edges brought together and welded by conventional techniques. US patent Application 2001/0008187 discloses a coaxial cable in which the outer conductor comprises an electro-conductive lacquer layer and preferably a metal layer applied to said lacquer layer. The central conductor provided with an electrically insulating layer is passed through a solution of an electro-conductive lacquer and preferably a thin metal layer is subsequently applied by means of electroless deposition in a liquid or by passing a cable through a solder bath of tin/lead.

US Patent Application 2004/0055153 discloses a method for producing a molding with an integrated conductor run. Three nozzles are disclosed located around a flexible tube for applying a particle beam in a conductor run by using cold gas spraying.

GB Patent 304 192 discloses ring shaped spray nozzles rotating around a cable to produce a uniform insulated coating. Further, it is disclosed that coatings of metals may be applied by this method.

Said cables and manufacturing methods thereof present disadvantages, for example, the manufacture of said cables is complex and slow and the cables are expensive due to the high quantity of conductive material used.

It is the object of the present invention to provide a process and apparatus for manufacturing structures guiding electromagnetic waves which solves the aforementioned problems.

The object is achieved by a process for manufacturing structures for guiding electromagnetic waves according to claim 1and an apparatus for manufacturing structures for guiding electromagnetic waves according to claim 6.

The manufacturing process according to the invention is based on the use of cold gas spraying for forming a thin, dense and adhesive conductive layer for transmission of radio frequency waves. Said conductive layer may be applied to form, for example, either the inner conductor conductive layer or the outer conductor of a coaxial cable. The outer conductor is realized by providing a cold gas sprayed layer of conductive material over the cable dielectric material.

A method and apparatus for cold gas spraying is already known from EP Patent Application 0 484 533, in which spray particles are accelerated to high speeds in a cold gas spray gun in a "cold" gas jet. The coating is formed by the impact of the particles with high kinetic energy on the work piece. Upon impact, the particles that do not melt in the "cold" gas jet form a dense and tightly adhering layer, the plastic deformation and the resulting local heat release providing for cohesion and adhesion of the sprayed layer to the work piece.

The use of cold gas spraying for manufacturing of structures guiding electromagnetic waves has advantages. Conductive layers produced with cold gas spraying do not need the use of vacuum, present good adhesion to metals or polymers and allow thin and dense structures providing a conductivity of at least 60 % the conductivity of the traditional solid metal conductor made of copper or silver. The manufacture costs of such cables and structures guiding electromagnetic waves with cold sprayed layers are thus lower due to the use of less conductive material e.g. copper or silver. The cables and other structures for guiding electromagnetic waves produced according to the invention take advantage of the observed fact that only little conductive material is needed for the transmission of radio frequency waves.

The invention also relates to an apparatus for manufacturing structures guiding electromagnetic waves. The apparatus according to the invention comprises preferably at least two wheels in charge of guiding and moving the cable and one or more spray nozzles in charge of applying the coating powder to said moving cable.. In a preferred embodiment only one spray nozzle is used which rotates around the cable.

The inventive process and apparatus of the invention enables the manufacture of coaxial cable in a simple, reliable and efficient manner. When the manufacturing process consists only on providing the outer conductor on the cable insulator then rates higher than two meters per minute are possible.

Further advantageous configurations of the invention emerge from the dependent claims, the following description and the drawings.

An embodiment example of the invention is now explained with the aid of Figures 1 to 4.
Figure 1 illustrates an apparatus for manufacturing structures for guiding electromagnetic waves according to the prior art.
Figure 2 shows a detailed view of the fixed spray nozzles used in Figure 1.
Figure 3 illustrates a preferred embodiment of an apparatus for manufacturing structures for guiding electromagnetic waves according to the invention.
Figure 4 shows a cross-sectional view of a structure for guiding electromagnetic waves.

Figure 1 shows an apparatus for manufacturing structures for guiding electromagnetic waves according to the prior art. The apparatus applied to the production of cables C for transmission of radio frequency electrical waves comprises two wheels W1 and W2 rotating at a certain velocity in order to move the cable at a certain line speed LS. The apparatus also comprises three nozzles N1 to N3 which apply the coating powder to the moving cable using cold gas spraying techniques.

The cable C is guided from one wheel to the other and passing a fixed structure comprising three spray nozzles. The choice of process parameters, especially the range of gas velocity may be on the range from 450 m/s to 1600m/s and resulting the velocity of powder P. Particle sizes in the spray may be chosen in the range from 2 µm up to 35 µm. The layer thickness is adjusted by setting the line speed LS and the spray gas velocity.

Although only a three fixed nozzle spray structure is shown, the number of nozzles may be varied from two to a larger number depending on the spray pattern of the nozzles used.

Figure 1 only shows a manufacturing process in which only one cold gas spray layer is applied to a cable C. In cases in which more than one cold gas spray layer shall be applied to the cable more wheels or more nozzle structures may be applied in series. As already mentioned, it is to be understood that the cold gas sprayed layer can be applied to different elements of the cable, i.e. a first layer could be applied for the inner conductor of the cable according to the invention, then such inner conductor would be covered, for example by extrusion or any other means, with a dielectric material and in a next step another conductive layer could be applied to the dielectric outer surface.; finally such cable structure could be covered by an outer protective jacket made of for example of a synthetic resin.

Figure 2 shows a detailed view of the three fixed spray nozzle configuration N1 to N3 which apply a cold gas layer to a tubular cable C. The cable C may be a tubular metal conductor over which a cold spray layer of high conductivity is being applied or may be a conductor with a dielectric coating made of e.g. polyethylene, polypropylene or polyetheretherketon over which a cold spray layer is applied.

Figure 3 shows a preferred embodiment of an apparatus for manufacturing structures for guiding electromagnetic waves according to the invention. The apparatus applied to the production of cables C for transmission of radio frequency electrical waves comprises two wheels W1 and W2 rotating at a certain velocity in order to move the cable at a certain line speed LS. The apparatus also comprises one nozzle N1 which applies the coating powder to the moving cable using cold gas spraying techniques. The nozzle N1 rotates in a certain direction R around the cable C in order to cover the whole surface of the cable. The high conductivity cold gas spray layer thickness depends on the line speed LS and the spray gas velocity and is adjusted by setting the speed of rotation R.

Although Figure 3 shows only one nozzle rotating around the cable C, it is understood that there may be rotating nozzle configuration variants in which two or more nozzles move around the cable by a certain angle.

Figure 4 shows a cross-sectional view of a structure for guiding electromagnetic waves 1 which is manufactured according to the method and by the apparatus as described above. In particular a coaxial cable comprising an inner conductor IC, a dielectric D having a wave-like outer surface and a metal conductive layer CL applied to said outer dielectric surface by means of a cold gas spraying process. Alternatively, other coaxial cable dielectric surface structures and forms can also be covered by cold gas spraying techniques and devices for applying conductive cold gas sprayed layer.

While the principles of the invention have been described above in connection with specific structures for guiding electromagnetic waves such as telecommunications cables, it is to be understood that the method and apparatus as described abovecould also be used for the production of antennas or other structures for guiding radio waves.

## Claims

1. Process for manufacturing structures for guiding electromagnetic waves (1), such as telecommunication cables, comprising at least a conductive layer (CL) for transmission of radio frequency waves, the conductive layer being formed by the use of cold gas spraying, **characterized in that** the conductive cold gas spray layeris applied by one or more spray nozzles (N1 to N3) rotating around a conductor or cable (C) moving with a certain line speed (LS) and the cold gas spray layer thickness is adjusted by setting the speed of rotation of the spray nozzles (N1 to N3).

2. The process of claim 1 **characterized in that** said conductive layer (CL) is applied over a metal tubular or solid conductor, such as an in inner conductor (IC) of a coaxial cable.

3. The process of claim 1 **characterized in that** said conductive layer (CL) is applied over a structure with a layer of dielectric material (D) such as polyethylene, polypropylene or polyetheretherketon.

4. The process of claim 1 **characterized in that** the conductive layer (CL) provides a conductivity of at least 60 % of the conductivity of the pure solid material.

5. The process of claim 1 **characterized in that** the conductive cold gas spray layer is applied by a fixed spray nozzle configuration, with at least two nozzles (N1 to N3), the spray nozzle configuration rotating around the conductor or cable (C).

6. Apparatus for manufacturing structures for guiding electromagnetic waves (1), such as telecommunication cables, comprising a least a conductive layer (CL) for transmission of radio frequency waves, and comprising
at least two wheels (W1 and W2) rotating at a certain velocity in order to move a conductor or cable (C) at a certain line speed (LS), and
at least one spray nozzle (N1) for applying a coating powder to the moving conductor or cable (C), said at least one spray nozzle (N1) comprising means for cold gas spraying.
**characterized in that**
the apparatus comprises means for rotating the one or more spray nozzles (N1 to N3) around the conductor or cabte (C) and means for setting the speed of rotation of the one or more spray nozzles (N1 to N3) to adjust the conductive cold gas spray layer thickness.

7. The apparatus of claim 8 **characterized in that** it comprises at least two spray nozzles (N1 to N3) located around the moving conductor or cable, the nozzles being in a fixed position and separated a certain angle from each other.

## Patentansprüche

1. Verfahren zur Herstellung von Strukturen zum Führen von elektromagnetischen Wellen (1) wie beispielsweise Telekommunikationskabel, umfassend zumindest eine leitfähige Schicht (CL) zur Übertragung von Funkfrequenzwellen, wobei die leitfähige Schicht durch Kaltgasspritzen gebildet wird, **dadurch gekennzeichnet, dass** die leitfähige Kaltgasspritzschicht durch eine oder mehrere Sprühdüsen (N1 bis N3), welche sich um einen Leiter oder ein Kabel (C) drehen und mit einer bestimmten Leitungsgeschwindigkeit (LS) bewegen, angebracht wird, und dass die Dicke der Kaltgasspritzschicht durch Einstellen der Drehgeschwindigkeit der Sprühdüsen (N1 bis N3) angepasst wird.

2. Verfahren nach Anspruch 1, **dadurch gekennzeichnet, dass** die besagte leitfähige Schicht (CL) über einem Metallrohr- oder Festkörperleiter wie beispielsweise einem Innenleiter (IC) eines Koaxialkabels angebracht wird.

3. Verfahren nach Anspruch 1, **dadurch gekennzeichnet, dass** die besagte leitfähige Schicht (CL) über einer Struktur mit einer Schicht aus dielektrischem Material (D) wie beispielsweise Polyethylen, Polypropylen oder Polyetheretherketon angebracht wird.

4. Verfahren nach Anspruch 1, **dadurch gekennzeichnet, dass** die leitfähige Schicht (CL) eine Leitfähigkeit von mindestens 60 % der Leitfähigkeit des reinen Festkörpermaterials gewährleistet.

5. Verfahren nach Anspruch 1, **dadurch gekennzeichnet, dass** die leitfähige Kaltgasspritzschicht durch eine feste Sprühdüsenkonfiguration mit mindestens zwei Düsen (N1 bis N3) angebracht wird, wobei sich die Sprühdüsenkonfiguration um den Leiter oder das Kabel (C) dreht.

6. Vorrichtung zur Herstellung von Strukturen zum Führen von elektromagnetischen Wellen (1) wie beispielsweise Telekommunikationskabel, umfassend zumindest eine leitfähige Schicht (CL) zur Übertragung von Funkfrequenzwellen, und umfassend
mindestens zwei Räder (W1 und W2), welche sich mit einer bestimmten Geschwindigkeit drehen, um einen Leiter oder ein Kabel (C) bei einer bestimmten Leitungsgeschwindigkeit (LS) zu bewegen, und
mindestens eine Sprühdüse (N1) zum Auftragen eines Beschichtungspulvers auf den sich bewegenden Leiter oder das sich bewegende Kabel (C), wobei die besagte mindestens eine Sprühdüse (N1) Mittel zum Kaltgasspritzen umfasst,
**dadurch gekennzeichnet, dass**
die Vorrichtung Mittel zum Drehen der einen oder mehreren Sprühdüsen (N1 bis N3) um den Leiter oder das Kabel (C) und Mittel zum Einstellen der Drehgeschwindigkeit der einen oder mehreren Sprühdüsen (N1 bis N3) zum Anpassen der Dicke der leitfähigen Kaltgasspritzschicht umfasst.

7. Vorrichtung nach Anspruch 8, **dadurch gekennzeichnet, dass** sie mindestens zwei Sprühdüsen (N1 bis N3) umfasst, welche um den sich bewegenden Leiter oder das sich bewegende Kabel angeordnet sind, wobei sich die Düsen in einer festen Position befinden und in einem bestimmten Winkel voneinander getrennt sind.

## Revendications

1. Procédé pour fabriquer des structures pour guider des ondes électromagnétiques (1), comme des câbles de télécommunication, comprenant au moins une couche conductrice (CL) pour la transmission d'ondes de radiofréquence, la couche conductrice étant formée par l'utilisation de projection par gaz froid, **caractérisé en ce que** la couche conductrice de projection par gaz froid est appliquée par une ou plusieurs buses de projection (N1 à N3) tournant autour d'un conducteur ou d'un câble (C) se déplaçant à une certaine vitesse de ligne (LS) et l'épaisseur de la couche de projection par gaz froid est ajustée en réglant la vitesse de rotation des buses de projection (N1 à N3).

2. Procédé selon la revendication 1 **caractérisé en ce que** ladite couche conductrice (CL) est appliquée sur un conducteur métallique tubulaire ou plein, comme un conducteur intérieur (IC) d'un câble coaxial.

3. Procédé selon la revendication 1 **caractérisé en ce que** ladite couche conductrice (CL) est appliquée sur une structure avec une couche de matériau diélectrique (D) comme du polyéthylène, du polypropylène ou du polyétheréthercétone.

4. Procédé selon la revendication 1 **caractérisé en ce que** la couche conductrice (CL) fournit une conductivité au moins 60 % égale à la conductivité du matériau solide pur.

5. Procédé selon la revendication 1 **caractérisé en ce que** la couche conductrice de projection par gaz froid est appliquée par une configuration de buses de projection fixes, avec au moins deux buses (N1 à N3), la configuration de buses de projection tournant autour du conducteur ou du câble (C).

6. Appareil pour fabriquer des structures pour guider des ondes électromagnétiques (1), comme des câbles de télécommunication, comprenant au moins une couche conductrice (CL) pour la transmission d'ondes de radiofréquence, et comprenant
au moins deux roues (W1 et W2) tournant à une certaine vitesse afin de déplacer un conducteur ou un câble (C) à une certaine vitesse de ligne (LS), et
au moins une buse de projection (N1) pour appliquer une poudre de revêtement sur le conducteur ou le câble (C) mobile, ladite au moins une buse de projection (N1) comprenant des moyens de projection par gaz froid.
**caractérisé en ce que**
l'appareil comprend des moyens pour tourner la ou les buses de projection (N1 à N3) autour du conducteur ou du câble (C) et des moyens pour régler la vitesse de rotation de la ou des buses de projection (N1 à N3) pour ajuster l'épaisseur de la couche conductrice de projection par gaz froid.

7. Appareil selon la revendication 8 **caractérisé en ce qu'**il comprend au moins deux buses de projection (N1 à N3) situées autour du conducteur ou du câble mobile, les buses étant dans une position fixe et séparées les unes des autres selon un certain angle.
